

UNITED STATES PATENT OFFICE

JOSEPH BECKER, OF PITTSBURGH, PENNSYLVANIA, ASSIGNOR TO THE KOPPERS COMPANY OF PITTSBURGH, PENNSYLVANIA, A CORPORATION OF PENNSYLVANIA

## PITCH-COKING PROCESS AND PRODUCT

No Drawing. Application filed October 16, 1919, Serial No. 330,988. Renewed March 21, 1924.

This invention relates generally to the coking of liquefiable bituminous material and has for a primary object a production of coke in a manner which substantially eliminates excess intumescence and ebullition of the material during the coking process, and to produce a coke for employment in metallurgical furnaces, which coke is formed from a mixture of pitch and a material that is substantially infusible at coking temperatures and whose residuum in the resultant coke is homologous with the material to be recovered in such furnaces. The process is, for instance, adapted for making coke for use in the making of electrodes for electric furnaces, especially as employed in the recovery of aluminum from its ores and contemplates the production of a coke of low-ash or low impurity as regards residues other than those homologous with the material to be recovered in such furnaces. Although the invention is especially applicable to the coking of pitch, it may readily be applied to other liquefiable bituminous materials, and it will be understood that the invention is not limited to the specific process nor to the specific application herein described as an illustrative example.

In carrying out the invention a proportion of pitch or other liquefiable bituminous material, is mixed with a proportion of a metallic compound that is infusible at coking temperature and checks foaming of the pitch and yet does not leave in the finished coke a residuum foreign to, nor introduce objectionable impurities into the material electrolytically treated in the electric furnace in which electrodes made of such coke are employed. The invention is of particular importance in the production of coke for the manufacture of carbon electrodes utilized in electric furnaces for the recovery of aluminum from its ores. Examples of such metallic compounds that are suitable for mixing with material, such as pitch, in order to carry out the coking process of the invention are alumina, i. e., the oxide of the metal aluminum, and bauxite or other ore containing the oxide of aluminum. The mixture thus formed, for example a mixture of pitch and bauxite, may then be charged into a coke oven retort of ordinary

type and subjected in the oven to the required coking heat. The coking process is carried on efficiently, without the usual difficulties encountered in the coking of ordinary pitch, or other analogous liquefiable bituminous materials, which when subjected to the high temperatures necessary for coking, frequently boil and intumesce violently. This foaming and intumescing of pitch materials in coke ovens results in a mechanical loss of a large proportion of the coke and produces conditions in the oven or retort which seriously interfere with the closures and outlets of the oven or retort. The coke resulting from a mixture of pitch and bauxite, for example, will be a highly homogeneous product, and of great value in the manufacture of carbon electrodes for aluminium furnaces which require the use of coke substantially ash-free or of low impurity as regards residues other than those homologous with the material to be recovered in such furnaces. This follows from the fact that the non-carbon residuum in such bauxite pitch coke will be the same material, bauxite, that is electrolytically treated in such furnaces.

An advantageous application of the above stated discovery is as follows: A proportion of ordinary pitch, or other liquefiable bituminous material is thoroughly mixed with a substantially equal proportion of bauxite. This mixture may then be charged into an oven and coked. Instead of employing raw bauxite in the mixture, a proportion of the coke produced from a similar mixture of pitch and bauxite, according to the above process, may be employed. This would result in a cyclic process for the manufacture of pitch coke. For example, a proportion of the coke produced from a mixture of pitch and bauxite, may be set aside and utilized for the production of a subsequent similar mixture. This would have the advantage that the coke produced would contain a relatively higher carbon content than would be the case if the coke be produced from a mixture of pitch and raw bauxite. Coke produced from a mixture of pitch and a substantially equal proportion of bauxite contains approximately 32% carbon and approximately 68% alumina. On the 100

other hand coke produced from a mixture of pitch and a substantially equal proportion of coke formed from a like previous mixture of coke and bauxite contains over 50% carbon and less than 50% alumina. The coke of higher carbon content is of course more desirable when employed for the manufacture of carbon electrodes for aluminium furnaces, inasmuch as it will not disintegrate as rapidly as the coke containing the higher alumina content.

The term "pitch" is used in the appended claims in a generic rather than a technically specific sense, and to include ebuliently liquefiable bituminous materials of the general nature of pitch; and my invention includes the treatment of such materials to produce a coke substantially ash-free or of low impurity as regards undesirable residues and yet remedy the coking difficulties hereinabove indicated.

The processes of the invention may be practiced in various ways, other than the particular embodiment that has been described for purposes of illustration, and still be within the scope and subject matter of the claims hereinafter made.

I claim:

1. In a pitch coking process; mixing a substantially equal proportion of pitch with a substantially equal portion of bauxite; and coking the mixture; substantially as specified.

2. In a pitch coking process for the production of coke for employment in electrodes of electrolytic furnaces; mixing pitch with a proportion of a material that is substantially infusible at coking temperatures and whose residuum in the resultant coke comprises alumina; and coking the mixture; substantially as specified.

3. A process which comprises coking a mixture containing pitch and a sufficient proportion of bauxite to prevent substantial foaming of the mixture during coking thereof.

4. A process which comprises coking a mixture containing pitch and a sufficient proportion of material comprising alumina to prevent substantial foaming of the mixture during coking thereof.

5. In a cyclic process for the manufacture of pitch coke, coking a mixture containing pitch and a sufficient proportion of bauxite to prevent substantial foaming of the mixture during coking thereof, making a mixture containing at least a portion of the resultant coke and pitch, and coking said mixture.

6. In a cyclic process for the manufacture of pitch coke, coking a mixture containing pitch and a sufficient proportion of material comprising alumina to prevent substantial foaming of the mixture during coking thereof, making a mixture containing at least a portion of the resultant coke and pitch, and coking said mixture.

7. In a cyclic process for the manufacture of pitch coke, mixing a substantially equal proportion of pitch with a substantially equal proportion of alumina, coking the mixture, making a mixture containing at least a proportion of the resultant coke and pitch, and coking said mixture.

8. A mixture containing pitch and a sufficient proportion of bauxite to prevent substantial foaming of the mixture during coking thereof.

9. A mixture containing pitch and a sufficient proportion of material comprising alumina to prevent substantial foaming of the mixture during coking thereof.

10. Coke made by coking a mixture of pitch and bauxite and substantially ash-free as regards residues other than bauxite.

11. Coke made by coking a mixture of pitch and material comprising alumina and substantially ash-free as regards residues other than alumina.

12. A process which comprises coking a mixture containing substantially ash-free bituminous material liquefiable by heat and a sufficient proportion of bauxite to prevent substantial foaming of the mixture during coking thereof.

13. A process which comprises coking a mixture containing substantially ash-free bituminous material liquefiable by heat and a sufficient proportion of material comprising alumina to prevent substantial foaming of the mixture during coking thereof.

14. A mixture containing substantially ash-free bituminous material liquefiable by heat and a sufficient proportion of bauxite to prevent substantial foaming of the mixture during coking thereof.

15. A mixture containing substantially ash-free bituminous material liquefiable by heat and a sufficient proportion of material comprising alumina to prevent substantial foaming of the mixture during coking thereof.

16. Coke made by coking a mixture of substantially ash-free bituminous material liquefiable by heat and bauxite and substantially ash-free as regards residues other than bauxite.

17. Coke made by coking a mixture of substantially ash-free bituminous material liquefiable by heat and material comprising alumina and substantially ash-free as regards residues other than alumina.

In testimony whereof I have hereunto set my hand this 7th day of October, 1919.

JOSEPH BECKER.